

## 1

3,206,405

**SYNTHETIC LUBRICANTS COMPRISING DEHYDROCONDENSATION PRODUCTS OF POLYESTERS**

Herbert L. Hepplewhite and Edward A. Oberright, Woodbury, and Robert H. Williams, Pennington, N.J., assignors to Socony Mobil Oil Company, Inc., a corporation of New York

No Drawing. Filed Jan. 2, 1962, Ser. No. 163,908  
14 Claims. (Cl. 252—56)

5  
10

This invention relates to the art of lubrication. More particularly, it is concerned with synthetic type lubricating oils comprising dehydrocondensation products of certain polyesters.

As is well known, mineral oils, which for many years had provided satisfactory lubrication for piston-engined aircraft, have proved to be inadequate for jet engines, due to the extreme ranges of temperatures to which the oil is subjected in jet aircraft. This need has been met by the development of synthetic-type lubricating oils, particularly the esters of dibasic acids. The latest types of turbo-jet and turbo-prop engines, however, have forced bearing and oil temperatures higher, i.e., up to 550–600° F. In order to provide adequate lubrication for these newer engines, increased viscosity of the lubricating oil at these higher operating temperatures is required. At the same time, the viscosity-temperature characteristics of the oil must be such as to permit starting the engine at temperatures below at least about –30° F. Thus, the pour point of the oil must be below –30° F. or lower.

In accordance with the present invention, it has been found that conventional polyester lubricating oils when reacted with certain organic peroxides form dehydrocondensation products having high temperature viscosities which are substantially higher than those of the polyesters themselves. At the same time the low temperature viscosity levels and pour points of the products can be maintained within reasonable limits. Thus, it has also been found that the viscosities of the products can be controlled by the amount of peroxide employed in the dehydrocondensation reaction whereby the products are suitable either as lubricating oils, *per se*, or (in the case of highly viscous products) as blending agents for conventional ester-type oils to improve the viscosity-temperature characteristics thereof. Also, the products of the invention exhibit good shear-resistance as opposed to conventional polymeric oil addends. It is, therefore, the primary object of this invention to provide a novel class of lubricating oils comprising dehydrocondensation products of polyesters.

It is also an object to provide novel lubricating oil compositions comprising blends of conventional ester oils and dehydrocondensed polyesters.

Other objects and advantages of the invention will appear from the following detailed description thereof.

The polyesters which may be dehydrocondensed in accordance with the invention may be any polyester having an abstractable hydrogen atom. Thus, di-, tri- and tetraesters of di-, tri- and tetra-carboxylic acids and di-tri-, tetra- and polyesters of glycols, triols and polyhydric al-

## 2

cohols may be employed. Non-limiting examples of suitable esters are the following:

Di-butyl phthalate  
Di-octyl adipate  
5 Di-2-ethylhexyl sebacate  
Di-2-ethylhexyl azelate  
Trimethylol propane trioctanoate  
Trimethylol propane tridecanoate  
Trimethylol butane hexanoate  
Pentaerythritol tetraoctanoate  
10 Pentaerythritol tetradodecanoate

The organic peroxides utilizable in the invention may be any organic peroxide or hydroperoxide which breaks down on heating to give free radicals. However, tertiary alkyl peroxides containing from 8 to about 20 carbon atoms, such as di-t-butyl peroxide, di-t-amyl peroxide, t-amyl, t-butyl peroxide and di-t-octyl peroxide, are particularly suitable.

The dehydrocondensation reaction is carried out by intermixing from about 5 to about 50 weight percent of the peroxide with the ester and heating the mixture for a period of from about 1 to about 10 hours at a temperature of from about 100° C. to about 200° C. Free alcohol formed in the reaction is then removed by distillation. The reaction can be carried out in one step utilizing relatively large amounts of peroxide, i.e., 15–20% or more, or it can be conducted in stages using relatively small amounts, such as about 5%, and repeating the reaction with this amount several times until a product having the desired viscosity is obtained. The latter procedure is useful in determining the amount of peroxide which will provide a product having a certain viscosity from a particular polyester, while the former procedure is generally the one used after such a determination has been made.

A full understanding of the invention will be had by reference to the following illustrative examples.

40

**EXAMPLE 1**  
*Dehydrocondensation of di-2-ethylhexyl sebacate*

A mixture of 500 grams of di-2-ethylhexyl sebacate and 45 25 grams of di-t-butyl peroxide were reacted under reflux at 135–145° C. for 5 hours. Tertiary butyl alcohol, formed during the reaction, was removed by distillation. A 100-gram sample was then removed from the reaction mixture. The reaction mixture was then subjected to reaction with four additional portions of peroxide under the same conditions as in the original reaction, the portion of peroxide added in each instance amounting to approximately 5% of the remaining reaction mixture. Table I shows the physical properties of the products obtained 55 in each of these reactions, numbered 1–5 in the table.

A separate reaction was also conducted under the conditions of the first of the preceding series of reactions, except that 18 weight percent of di-t-butyl peroxide was reacted all at once with the di-2-ethylhexyl sebacate. The properties of the product of this reaction (Reaction No. 60 6) are also given in Table I.

It will be seen from Table I that the viscosity of the dehydrocondensation product increases in proportion to 65 the amount of peroxide employed in the reaction. How-

ever, the pour point of the products is not increased over that of the original ester.

TABLE I.—PROPERTIES OF DEHYDROCONDENSED DI-2-ETHYLHEXYL SEBACATE

|                             | Unreacted polyester | Product of Reaction No. 1 | Product of Reaction No. 2 | Product of Reaction No. 3 | Product of Reaction No. 4 | Product of Reaction No. 5 | Product of Reaction No. 6 |
|-----------------------------|---------------------|---------------------------|---------------------------|---------------------------|---------------------------|---------------------------|---------------------------|
| KV at 400° F., cs.          | 1.08                | 1.24                      | 1.48                      | 1.77                      | 2.07                      | 2.23                      | 2.00                      |
| KV at 210° F., cs.          | 3.31                | 4.12                      | 5.22                      | 6.75                      | 8.81                      | 9.65                      | 8.32                      |
| KV at 100° F., cs.          | 12.57               | 17.30                     | 24.43                     | 34.88                     | 50.17                     | 56.81                     | 45.78                     |
| KV at -40° F., cs.          | 1,426               | 2,625                     | 4,969                     | 9,364                     | 17,740                    | 22,340                    | 14,910                    |
| ASTM slope                  | -0.71               | -0.69                     | -0.66                     | -0.64                     | -0.61                     | -0.61                     | -0.62                     |
| Percent recovery per treat. | 99.3                | 99.4                      | 99.4                      | 99.1                      | 98.2                      | 97.8                      | 97.8                      |
| Flash point, COC, ° F.      | 465                 | 450                       | 455                       | 460                       | 450                       | 440                       | 440                       |
| API gravity                 | 23.3                | 21.8                      | 21.6                      | 20.9                      | 19.7                      | 20.9                      | 20.4                      |
| Neutralization No.          | 0.17                | 0.14                      | 0.44                      | 0.59                      | 0.66                      | 0.68                      | 0.60                      |
| Pour point, ° F.            | <-65                | <-65                      | <-65                      | <-65                      | <-65                      | <-65                      | <-65                      |

## EXAMPLE 2

## Dehydrocondensation of trimethylol propane trioctanoate

A mixture of 503 grams of trimethylol propane tri-octanoate and 25 grams of di-t-peroxide were reacted under reflux at 140–150° C. for 6 hours. Tertiary butyl alcohol, formed during the reaction, was removed by distillation. A 100-gram sample was then removed from the reaction mixture. The reaction mixture was then subjected to reaction with three additional portions of peroxide under the same conditions as the original reaction. A sample of the reaction mixture (product) was taken after each reaction. The portion of peroxide added in each instance amounted to approximately 5%, by weight, of the remaining reaction mixture. The physical properties of the products of these four reactions are given in Table II.

Here again, it is seen that the viscosities of the products are greater than those of the original ester and that the viscosities increase in proportion to the amount of peroxide used. At the same time, however, the pour point of the products remains unchanged.

TABLE II.—PROPERTIES OF DEHYDROCONDENSED TRIMETHYLOL PROPANE TRIOCTANOATE

|                    | Unreacted polyester | Product of Reaction No. 1 | Product of Reaction No. 2 | Product of Reaction No. 3 | Product of Reaction No. 4 |
|--------------------|---------------------|---------------------------|---------------------------|---------------------------|---------------------------|
| KV at 400° F.      | 1.12                | 1.37                      | 1.66                      | 2.13                      | 2.81                      |
| KV at 210° F.      | 4.21                | 5.33                      | 6.98                      | 10.00                     | 14.51                     |
| KV at 100° F.      | 19.60               | 28.42                     | 41.62                     | 65.42                     | 113.8                     |
| KV at -40° F.      | 4,067               | 8,534                     | 18,444                    | 48,928                    | —                         |
| API gravity        | 16.8                | 15.9                      | 15.3                      | 14.1                      | 13.7                      |
| Neutralization No. | 0.10                | 0.76                      | 1.1                       | 1.2                       | 1.2                       |
| Pour point, ° F.   | <-30                | <-30                      | <-30                      | <-30                      | <-30                      |
| Flash point, ° F.  | 470                 | 480                       | 485                       | 495                       | 500                       |

## EXAMPLE 3

## Dehydrocondensation of trimethylol propane tripelargonate

In this example the trimethylol propane tripelargonate was reacted for 6 hours with 15%, by weight, of di-t-butyl peroxide at 135–150° C. The t-butyl alcohol formed in the reaction was removed by distillation. The properties of the original ester and the dehydrocondensate product are shown in Table III.

TABLE III.—PROPERTIES OF DEHYDROCONDENSATE OF TRIMETHYLOL PROPANE TRIPELARGONATE

|                    | Unreacted ester | Dehydrocondensate product |
|--------------------|-----------------|---------------------------|
| KV at -40° F.      | 5,130           | 50,000                    |
| KV at 100° F.      | 24.13           | 116.2                     |
| KV at 210° F.      | 4.93            | 15.53                     |
| KV at 400° F.      | 1.42            | 3.11                      |
| Pour point, ° F.   | -65             | -55                       |
| Neutralization No. | 0.01            | 0.28                      |
| Flash point, ° F.  | 525.0           | 530                       |

## EXAMPLE 4

## Dehydrocondensation of "Hercolube 600"

A mixture 502 grams of "Hercolube 600" (a mixed C<sub>8</sub>–C<sub>12</sub> fatty acid ester of pentaerythritol) and 25 grams of di-t-butyl peroxide were reacted under reflux at 140° C. to 150° C. for 6 hours. Tertiary butyl alcohol, formed during the reaction, was removed by distillation. A 100-gram sample was removed from the reaction mixture. The reaction mixture was subjected to 3 further reactions

as in Examples 1 and 2, i.e., by adding fresh portions of peroxide amounting in each instance to about 5%, by weight, of the reaction mixture after withdrawal of samples. The physical properties of the products are given in Table IV.

It is seen that as in Examples 1–3, the viscosities of the products increase in proportion to the amount of peroxide reacted with the ester. However, in this case it is noted that the pour point of the product of the fourth peroxide reaction shows a rise over that of the ester.

TABLE IV.—DEHYDROCONDENSATION OF "HERCOLUBE 600" (MIXED C<sub>8</sub>–C<sub>12</sub> ACID ESTER OF PENTAERYTHRITOL)

|                    | Unreacted polyester | Product of Reaction No. 1 | Product of Reaction No. 2 | Product of Reaction No. 3 | Product of Reaction No. 4 |
|--------------------|---------------------|---------------------------|---------------------------|---------------------------|---------------------------|
| KV at 400° F.      | 1.27                | 1.71                      | 2.32                      | 3.48                      | 6.04                      |
| KV at 210° F.      | 4.95                | 7.45                      | 11.46                     | 20.21                     | 41.63                     |
| KV at 100° F.      | 26.42               | 46.80                     | 86.82                     | 185.8                     | 478.2                     |
| KV at -40° F.      | 8,160               | 28,787                    | 100×10 <sup>6</sup>       | 200×10 <sup>6</sup>       | —                         |
| API gravity        | 9.8                 | 9.0                       | 7.8                       | 6.8                       | 6.4                       |
| Neutralization No. | 0.17                | 0.22                      | 0.40                      | 0.48                      | 0.87                      |
| Pour point, ° F.   | <-30                | <-30                      | <-30                      | <-30                      | -10                       |
| Flash point, ° F.  | 495                 | 515                       | 500                       | 515                       | 515                       |
| Molecular weight   | 555                 | 660                       | 780                       | 1,200                     | —                         |

5  
EXAMPLE 5

*Preparation of blending agent from "Hercolube 600"*

"Hercolube 600" was refluxed with 25 weight percent of di-t-butyl peroxide at 140–150° C. for several hours. In the course of stripping the product, a gel was formed. Liquid product was extracted with toluene, in which the gel is insoluble. This material (extract) was used as a blending stock in di-2-ethylhexyl sebacate, trimethylol propane trioctanoate and "Hercolube 600." Properties of the blends, as well as Sonic Oscillator shear data, are given in Table V.

It will be seen that the dehydrocondensed ester is highly advantageous as a blending stock for the ester-type oils, since it substantially increases both the viscosity and viscosity index of the base ester oil. It is seen further that the 10% treated-ester blend does not significantly detract from the shear stability of the (di-2-ethylhexyl sebacate) oil.

Results similar to those shown in Table V are attained with blends of the products in conventional ester oils other than di-2-ethylhexyl sebacate. As is well known, these ester oils are derived from either (a) monohydric aliphatic alcohols, such as butyl, iso-butyl, octyl, decyl, dodecyl and tetradecyl alcohol, and aliphatic dicarboxylic acids, such as adipic, pimelic, suberic, azelaic and sebacic acid, or (b) polyhydric alcohols, such as ethylene glycol, trimethylol propane, trimethylol butane, pentaerythritol, etc., and monocarboxylic acids, such as acetic, valeric, decanoic, myristic, stearic, etc.

TABLE V.—PROPERTIES OF "HERCOLUBE 600" DEHYDROCONDENSATE<sup>1</sup> BLENDS

| Base fluid                       | Dehydrocondensate, wgt. percent | KV at -40° F. | KV at 100° F. | KV at 210° F. | VI  |
|----------------------------------|---------------------------------|---------------|---------------|---------------|-----|
| Di-2-ethylhexyl sebacate         | 0                               | 1,426         | 12.55         | 3.31          | 154 |
|                                  | 5                               | 2,155         | 18.02         | 4.58          | 185 |
|                                  | 10                              | 3,225         | 25.46         | 6.28          | 173 |
|                                  | 15                              | 5,079         | 36.23         | 8.55          | 166 |
| Trimethylol propane trioctanoate | 0                               | 4,067         | 19.60         | 4.21          | 139 |
|                                  | 5                               | 6,435         | 28.09         | 5.74          | 151 |
|                                  | 10                              | 10,140        | 40.18         | 7.48          | 152 |
|                                  | 15                              | 15,042        | 57.75         | 11.01         | 150 |
| "Hercolube 600"                  | 0                               | 8,180         | 26.42         | 4.95          | 129 |
|                                  | 5                               | 14,180        | 39.06         | 7.21          | 143 |
|                                  | 10                              | 23,111        | 56.45         | 9.86          | 143 |
|                                  | 15                              | 33,596        | 83.21         | 13.98         | 143 |

Sonic Oscillator Shear Test:<sup>2</sup>

Sample=10 wgt. percent of "Hercolube 600" dehydrocondensate in di-2-ethylhexyl sebacate.

KV at 210° F. Original=6.23

Final=5.92

Percent Change=−5

(1) "Hercolube 600" dehydrocondensate: KV at 210° F.=748.6.

(2) ASTM Proposed Test Method, Preprint 35-S, 1961, Appendix XII, page 61.

EXAMPLE 6

*Dehydrocondensation of fluoroalkyl camphorate*

A mixture of 202 grams of Du Pont Stable Lubricant No. 316, a fluoroalkyl camphorate (a diester of camphoric acid and the fluoro alcohol,  $H(CF_2)_6CH_2OH$ ) and 18 grams of di-t-butyl peroxide was refluxed for 16 hours. Light products were removed by distillation and unreacted starting material was removed by vacuum distillation. The yield of product was 37 grams (18.5% based on the starting ester). The properties are given in Table VI. It will be seen that the product has a viscosity and flash point substantially higher than the original ester.

TABLE VI.—PROPERTIES OF FLUOROALKYL CAMPHORATE DEHYDROCONDENSATION PRODUCT

|                  | Unreacted ester | Dehydrocondensation product |
|------------------|-----------------|-----------------------------|
| KV at 100° F.    | 115.5           | 8,114                       |
| KV at 210° F.    | 8.22            | 97.96                       |
| Flash point, °F. | 460             | 525                         |

As shown in Tables I–IV, the neutralization number (N.N.) of the dehydrocondensation product in some instances is slightly higher than that of the starting polyester. However, this increase in N.N. can be eliminated by simple percolation over a suitable adsorbent, such as alumina or florilis.

Table VII shows the results obtained by the percolation treatment of a dehydrocondensed trimethylol propane tripelargonate ester. It will be seen that the product which was not subjected to percolation had an N.N. of 0.28, but that the N.N. of the percolated product with or without thermal treatment (columns 2 and 3) was lowered to substantially that of the original ester.

It has been found also that reaction of the starting ester with over about 10%, by weight, of peroxide provides a product of somewhat lower thermal stability than that of the starting ester. However, this may be overcome by subjecting the product to a simple thermal treatment. This involves simply heating the product to a temperature of, say, 400–600° F. in a nitrogen atmosphere. Table VIII shows the effect of the thermal treatment on the thermal stability of a dehydrocondensed trimethylol alkane tripelargonate. It will be seen from the table that percolation alone has only a minor effect on the thermal stability of the product, while heat-treating results in a large improvement in thermal stability. Percolation used after heat-treating removes acidic decomposition products and improves the color of the product.

TABLE VII.—EFFECT OF THERMAL TREATMENT AND/OR PERCOLATION ON PHYSICAL PROPERTIES OF DEHYDROCONDENSED TRIMETHYLOL PROPANE TRIPELARGONATE

|                    | 15% di-t-butyl peroxide reaction product |            |                                           |
|--------------------|------------------------------------------|------------|-------------------------------------------|
|                    | No treatment                             | Percolated | Thermally-treated percolated <sup>1</sup> |
| 35                 |                                          |            |                                           |
| KV at -40° F.      | 50,000                                   |            | 30,000                                    |
| KV at 100° F.      | 116.2                                    | 100.6      | 60.24                                     |
| KV at 210° F.      | 15.53                                    | 14.44      | 9.48                                      |
| KV at 400° F.      | 3.11                                     |            | 2.1                                       |
| Pour point, °F.    | −55                                      |            | <−65                                      |
| Neutralization No. | 0.28                                     | 0.00       | 0.05                                      |
| Flash point, °F.   | 530                                      |            | 525                                       |

<sup>1</sup> Heated at 536° F. for 24 hours under nitrogen and percolated over clay and alumina.

TABLE VIII.—THERMAL STABILITY<sup>1</sup> OF TREATED AND UNTREATED DEHYDROCONDENSED TRIMETHYLOL PROPANE TRIPELARGONATE

|                               | 15% di-t-butyl peroxide reaction product |            |                                               |
|-------------------------------|------------------------------------------|------------|-----------------------------------------------|
|                               | No treatment                             | percolated | Thermally treated and percolated <sup>2</sup> |
| 50                            |                                          |            |                                               |
| Weight loss, percent change   | 0.3                                      | 0.0        | 0.4                                           |
| KV at 100° F., percent change | −29.7                                    | −23.2      | +3.3                                          |
| KV at 210° F., percent change | −24.7                                    | −22.0      | +0.8                                          |
| Neutralization Number         | 2.5                                      | 1.6        | 0.9                                           |
| 55                            |                                          |            |                                               |

<sup>1</sup> Test Method: Sample heated to 536° F. in nitrogen atmosphere for 24 hours.

<sup>2</sup> Heated at 536° F. for 24 hours under nitrogen and percolated over clay and alumina.

It will be seen that the invention (1) provides polyester dehydrocondensation products having viscosities and low temperature characteristics which make them desirable lubricating oils for high temperature application, such as jet engine lubricants and (2) that these products are highly advantageous blending agents for conventional ester lubricating oils. It will be understood that the amount of the dehydrocondensation product added to an ester base oil can vary over a wide range, depending upon the viscosity of the particular product used and the viscosity desired in the finished blend. Thus, the products, being lubricating oils of themselves, may comprise either

a major or a minor proportion of the finished oil blends. From the standpoint of increasing the viscosity and/or viscosity index of the ester-base oil, however, the amount of dehydrocondensation product employed will generally be no greater than about 40 weight percent and may be as little as 1 weight percent, based on the total composition.

The lubricating oil compositions of the invention may contain additives normally added to lubricating oil for the purpose of improving the various characteristics thereof, such as antioxidants, detergents, extreme pressure agents, anti-wear agents, metal deactivators, etc.

Although the invention has been illustrated herein by means of specific examples and embodiments thereof, it is not intended that the scope of the invention be limited in any way thereby except as defined in the following claims.

We claim:

1. A lubricating oil comprising a dehydrocondensation product prepared by reacting (a) a polyester derived from a carboxylic acid, selected from the group consisting of mono- and polycarboxylic acids, said acids containing from about 2 to about 20 carbon atoms exclusive of carboxyl carbons, and an alcohol, selected from the group consisting of mono- and polyhydroxy alcohols, said alcohol containing from about 2 to about 20 carbon atoms with (b) from about 5% to about 50%, by weight, based on the polyester, of a di-tertiary alkyl peroxide containing from about 8 to about 20 carbon atoms, at a temperature of from about 100° C. to about 200° C. to form a dehydrocondensation product of said polyester and removing free alcohol formed in the reaction from the dehydrocondensation product.

2. A lubricating oil comprising a dehydrocondensation product prepared by reacting di-2-ethylhexyl sebacate with from about 5% to about 50%, by weight, based on the weight of the di-2-ethylhexyl sebacate, of di-tertiary-butyl peroxide, at a temperature of from about 100° C. to about 200° C., to form a dehydrocondensation product of di-2-ethylhexyl sebacate and removing free di-tertiary-butyl alcohol formed in the reaction from the dehydrocondensation product.

3. A lubricating oil comprising a dehydrocondensation product prepared by reacting trimethylol propane trioctanoate with from about 5% to about 50%, by weight, based on the weight of the trimethylol propane trioctanoate, of di-tertiary-butyl peroxide, at a temperature of from about 100° C. to about 200° C., to form a dehydrocondensation product of trimethylol propane trioctanoate and removing free di-tertiary-butyl alcohol formed in the reaction from the dehydrocondensation product.

4. A lubricating oil comprising a dehydrocondensation product prepared by reacting trimethylol propane tripelargonate with from about 5% to about 50%, by weight, based on the weight of the trimethylol propane tripelargonate, of di-tertiary-butyl peroxide, at a temperature of from about 100° C. to about 200° C., to form a dehydrocondensation product of trimethylol propane tripelargonate and removing free di-tertiary-butyl alcohol formed in the reaction from the dehydrocondensation product.

5. A lubricating oil comprising a dehydrocondensation product prepared by reacting a mixed C<sub>8</sub>-C<sub>12</sub> carboxylic acid ester of pentaerythritol with from about 5% to about 50%, by weight, based on the weight of said ester, of di-tertiary-butyl peroxide, at temperature of from about 100° C. to about 200° C., to form a dehydrocondensation product of the mixed C<sub>8</sub>-C<sub>12</sub> carboxylic acid ester of pentaerythritol and removing free di-tertiary-butyl alcohol formed in the reaction from the dehydrocondensation product.

6. A lubricating oil composition comprising a blend of a conventional ester oil and a dehydrocondensation product prepared by reacting (a) a polyester derived from a carboxylic acid, selected from the group consisting of

mono- and polycarboxylic acids, said acids containing from about 2 to about 20 carbon atoms exclusive of carboxyl carbons, and an alcohol, selected from the group consisting of mono- and polyhydroxy alcohols, said alcohol containing from about 2 to about 20 carbon atoms with (b) from about 5% to about 50%, by weight, based on the polyester of a di-tertiary alkyl peroxide containing from about 8 to about 20 carbon atoms, at a temperature of from about 100° C. to about 200° C. to form a dehydrocondensation product of said polyester and removing free alcohol formed in the reaction from the dehydrocondensation product.

7. A lubricating oil composition comprising a blend of a conventional ester oil and a dehydrocondensation product prepared by reacting di-2-ethylhexyl sebacate with from about 5% to about 50%, by weight, based on the weight of the di-2-ethylhexyl sebacate, of di-tertiary-butyl peroxide, at a temperature of from about 100° C. to about 200° C., to form a dehydrocondensation product of di-2-ethylhexyl sebacate and removing free di-tertiary-alcohol formed in the reaction from the dehydrocondensation product.

8. A lubricating oil composition comprising a blend of a conventional ester oil and a dehydrocondensation product prepared by reacting trimethylol propane trioctanoate with from about 5% to about 50%, by weight, based on the weight of the trimethylol propane trioctanoate, of di-tertiary-butyl peroxide, at a temperature of from about 100° C. to about 200° C., to form a dehydrocondensation product of trimethylol propane trioctanoate and removing free di-tertiary-butyl alcohol formed in the reaction from the dehydrocondensation product.

9. A lubricating oil composition comprising a blend of a conventional ester oil and a dehydrocondensation product prepared by reacting trimethylol propane tripelargonate with from about 5% to about 50%, by weight, based on the weight of the trimethylol propane tripelargonate, of di-tertiary-butyl peroxide, at a temperature of from about 100° C. to about 200° C., to form a dehydrocondensation product of trimethylol propane tripelargonate and removing free di-tertiary-butyl alcohol formed in the reaction from the dehydrocondensation product.

10. A lubricating oil composition comprising a blend of a conventional ester oil and a dehydrocondensation product prepared by reacting a mixed C<sub>8</sub>-C<sub>12</sub> carboxylic acid ester of pentaerythritol with from about 5% to about 50%, by weight, based on the weight of said ester, of di-tertiary-butyl peroxide, at a temperature of from about 100° C. to about 200° C., to form a dehydrocondensation product of the mixed C<sub>8</sub>-C<sub>12</sub> carboxylic acid ester of pentaerythritol and removing free di-tertiary-butyl alcohol formed in the reaction from the dehydrocondensation product.

11. A lubricating oil as defined in claim 1 which has been improved as to its thermal stability by heating to a temperature of from about 400° F. to about 600° F. in a nitrogen atmosphere.

12. The lubricating oil composition of claim 6, wherein the amount of dehydrocondensation product blended with the conventional ester oil is from about 1% to 40%, by weight, of total composition.

13. A lubricating oil comprising a dehydrocondensation product prepared by reacting a polyester having an abstractable hydrogen atom with from about 5% to about 50%, by weight, based on the polyester, of a di-tertiary alkyl peroxide containing from about 8 to about 20 carbon atoms, at a temperature of from about 100° C. to about 200° C. to form a dehydrocondensation product of said polyester and removing free alcohol formed in the reaction from the dehydrocondensation product.

14. A lubricating oil composition comprising a blend of a conventional ester oil and a dehydrocondensation product prepared by reacting a polyester having an abstractable hydrogen atom with from about 5% to about 50%, by weight, based on the polyester of a di-tertiary

alkyl peroxide containing from about 8 to about 20 carbon atoms, at a temperature of from about 100° C. to about 200° C. to form a dehydrocondensation product of said polyester and removing free alcohol formed in the reaction from the dehydrocondensation product.

|           |       |                 |       |           |
|-----------|-------|-----------------|-------|-----------|
| 2,808,418 | 10/57 | Harrison        | ----- | 260—404.8 |
| 2,820,014 | 1/58  | Hartley et al.  | ----- | 252—56    |
| 2,839,571 | 6/58  | Johnston et al. | ----- | 260—485   |
| 2,961,406 | 11/60 | McNeil et al.   | ----- | 252—56    |
| 2,993,860 | 7/61  | Critchley       | ----- | 252—57    |

## FOREIGN PATENTS

|         |      |                |
|---------|------|----------------|
| 591,543 | 8/47 | Great Britain. |
|---------|------|----------------|

## References Cited by the Examiner

## UNITED STATES PATENTS

|           |       |              |       |           |    |                                           |
|-----------|-------|--------------|-------|-----------|----|-------------------------------------------|
| 2,429,219 | 10/47 | Cowan        | ----- | 260—407 X | 10 | DANIEL E. WYMAN, <i>Primary Examiner.</i> |
| 2,801,263 | 7/57  | Hasek et al. | ----- | 260—485   |    | JULIUS GREENWALD, <i>Examiner.</i>        |

UNITED STATES PATENT OFFICE  
CERTIFICATE OF CORRECTION

Patent No. 3,206,405

September 14, 1965

Herbert L. Hepplewhite et al.

It is hereby certified that error appears in the above numbered patent requiring correction and that the said Letters Patent should read as corrected below.

Column 3, line 21, for "di-t-peroxide" read -- di-t-butyl peroxide --; column 6, TABLE VII, in the heading to columns 2, 3 and 4, for "15% di-t-butyl perTxide" read -- 15% di-t-butyl peroxide --; column 8, line 25, for "preparted" read -- prepared --.

Signed and sealed this 24th day of May 1966.

(SEAL)

Attest:

ERNEST W. SWIDER

Attesting Officer

EDWARD J. BRENNER

Commissioner of Patents